

## UNITED STATES PATENT OFFICE.

ROBERT JOHN, OF NEW YORK, N. Y., ASSIGNOR TO DAYLIGHT FILM CORPORATION, A CORPORATION OF NEW YORK.

## PROCESS OF PHOTOGRAPHIC REPRODUCTION DIRECTLY FROM A NEGATIVE.

No Drawing.

Application filed October 2, 1919. Serial No. 327,890.

*To all whom it may concern:*

Be it known that I, ROBERT JOHN, a citizen of the United States, residing at New York, in the county of New York and State of New York, have invented a certain new and useful Process of Photographic Reproduction Directly from a Negative, of which the following is a specification.

My invention relates to a process of photographic reproduction directly from a negative and has for its object to produce a printing surface containing a photographic record of lights and shades from which copies can be made by a dye or ink contact transfer process. An illustrative dye contact transfer process is disclosed in patent to Shepherd and Bartlett, No. 728,310, granted May 19, 1903, for photographic printing, and an illustrative ink contact transfer process is disclosed in Cassell's Cyclopaedia of Photography, Cassell & Co., New York, 1912, at page 124 under the title "Collo-type," it being understood, however, that the processes thus illustrated do not use a printing plate having the novel and beneficial characteristics of the printing plate disclosed herein. Although for general purposes the preferred method is to obtain the photographic record for the printing surface from a completed negative, it may be obtained by direct exposure, as, for example, in a camera, as described herein. The printing surface when treated with dye or ink also may be used in the same manner as a positive, either for direct view, or with reflected light, or with transmitted light as in a projecting machine.

The invention is applicable to monochromatic, polychromatic, or natural color photography both in still photography and in motion picture photography. The term "color" is intended to include "black," which sometimes technically is designated as an absence of color.

In the embodiment of my invention chosen for purposes of illustration, a sensitized emulsion such as a silver salt emulsion is exposed, as, for example, in a camera, to the action of light modified by the lights and shades of the object which it is desired to reproduce. The silver salt emulsion may be carried or mounted on any desired support, either opaque, translucent, or transparent, but preferably is mounted on a transparent

carrier such, for example, as glass or a cellulose base, in order that the silver salt emulsion may be exposed to the modified light through its transparent carrier.

The exposed emulsion then is treated by any ordinary developer having no tanning or hardening action on the emulsion, after which it is rinsed thoroughly in cold water and exposed again, preferably through its transparent carrier, to an actinic light. At this stage, therefore, the unhardened emulsion has two images,—one the usual photographic reversed negative image in metallic silver, and the other a latent image in undeveloped, light-affected, sensitized particles correctly reproducing the object photographed the same as would a positive made in usual manner from a negative. It then is necessary only to harden the emulsion adjacent the undeveloped, light-affected, sensitized particles and remove the unhardened emulsion in order to obtain the desired printing surface on the original negative.

One process of hardening the emulsion adjacent the undeveloped, light-affected, sensitized particles is described in my copending application for Letters Patent Serial No. 313,237, filed July 25, 1919, which eventuated into Patent No. 1,374,853, granted April 12, 1921. In the embodiment of that process described in said application, the emulsion is treated by a developing solution containing a hardening or tanning agent which renders insoluble or unremovable the emulsion adjacent its light-affected, light-sensitive content, the effect of which agent is controlled or limited selectively by the presence of varying quantities of a neutralizing agent, after which the soluble or removable portions of emulsion are removed in any desired manner, as, for example, by melting with warm water.

The result of the above treatment is the production of what may be termed a printing surface having novel characteristics and beneficial properties never before attained.

The most important of the novel characteristics is a printing surface comprising granules or great numbers of photographically formed, extremely minute, individual protuberances which are distributed and grouped irregularly so as to represent photographic lights and shades.

The most important of the beneficial prop-

erties is that such a printing surface when treated with a dye, ink, or other coloring matter, will absorb or take up or carry the coloring matter within a few seconds, and 5 when thus treated and placed in contact with a substance which is to carry the final reproduction, such for example as a gelatin, will give up its coloring matter practically instantaneously and produce on said gelatin 10 an exact and perfect reproduction. This speedy result, which is novel and was impossible of attainment before the present invention, is of prime importance in the production of motion picture positives from 15 motion picture negatives, although the saving of time and the superior results obtainable in still photography also are important. The printing plate or film, moreover, when treated with coloring matter, may be used 20 as a positive if reproductions are not desired.

A sample formula for a developing solution containing a hardening or tanning agent the effect of which is controlled and 25 limited selectively by the presence of varying quantities of a neutralizing agent is as follows:

|                                             |                  |
|---------------------------------------------|------------------|
| Water                                       | 8.5 ounces.      |
| Pyrogallic acid                             | 11 grains.       |
| Metol (monomethyl paramido-phenol sulphate) | 9 grains.        |
| Potassium bromide                           | 4 grains.        |
| Sodium carbonate                            | 200 grains.      |
| Sodium sulphite                             | 40 to 60 grains. |

In the above sample formula the hardening or tanning agent is pyrogallic acid, and the controlling and limiting agent is sodium sulphite which may be varied in amount 40 selectively within limits to obtain the desired result. It is well known that pyrogallic acid also is a developing agent and that sodium sulphite is a preservative adapted to prevent oxidation of the pyrogallic acid in solution. Other hardening and tanning agents and other neutralizing agents may be used, the above formula representing one developing solution by which the process 45 may be carried out. Potassium bromide, for example, also has a certain controlling and limiting effect. The main difference between the above sample formula and standard developing formulas is in the amount of sodium sulphite used. In standard formulas the amount of sodium sulphite used is so greatly in excess of the amount used in the above sample formula that the tanning or hardening effect of the pyrogallic acid is entirely neutralized or overcome. In 50 the sample formula, the sodium sulphite merely controls and limits the hardening effect of the pyrogallic acid. It is of course understood by those skilled in the art that when a thick layer of emulsion is treated, or 55 when the exposure is through the trans-

parent carrier, it is advisable, in order to accelerate the action of the pyrogallic acid, to use larger quantities of an accelerator such, for example, as sodium carbonate or its equivalents than when the emulsion layer 70 is thin or exposed on its face. When larger quantities of sodium carbonate thus are used, it is necessary to increase the amount of sodium sulphite. The above sample formula is for treatment of an emulsion exposed through its transparent carrier and therefore contains a comparatively large amount of sodium carbonate with an increased amount of sodium sulphite. In order 75 to obtain the desired printing surface, however, the amount of sodium sulphite in the process disclosed herein is much less than would be used in a developing solution for the usual development of the particular emulsion layer to be treated. Although it is 80 preferable for reasons of convenience to embody the selectively controlled hardening agent in the developer solution, it may be used separately if desired, by such modification of the developer solution as will prevent such a hardening of the emulsion as 85 will prevent the selective hardening desired.

It is believed that the hardening or tanning effect of the pyrogallic acid exerts its action first adjacent the so-called latent 90 image, or in other words, on the portions of emulsion adjacent the particles of silver salts affected by the exposure light and converted by the developer into metallic silver. Thus in a silver bromide film, the throwing off of the bromide from a light-affected silver bromide particle in the developing process, probably reacts with the pyrogallic acid to harden or tan or render insoluble or unremovable the adjacent emulsion. Thus in 100 the embodiment chosen for purposes of illustration, the reaction products from the chemical effects of the developer solution, are believed to react with the selectively controlled hardening agent, the essential result being a hardened emulsion surface corresponding to the lights and shades to be reproduced which will acquire and give up any desired color in a comparatively short time. By controlling the hardening or tanning effect of the pyrogallic acid as above 105 set forth, only the particles of emulsion adjacent the said light-affected particles of silver salts are hardened, the relative proportions of the hardening agent (whether or not accelerated by an accelerating agent) and of the neutralizing agent being such as to control selectively the effective area of influence of the hardening agent. The unhardened portions, as stated above, then may 110 be removed in any desired manner as by placing the emulsion in warm water which causes the unhardened or soluble portions to soften and melt away from the hardened or 115 insoluble portions so that the hardened 120

75  
80  
85  
90  
95  
100  
105  
110  
115  
12080  
85  
90  
95  
100  
105  
110  
115  
12090  
95  
100  
105  
110  
115  
120100  
105  
110  
115  
120105  
110  
115  
120110  
115  
120115  
120120  
125

emulsion alone will remain in the form of extremely minute, individual protuberances which are distributed and grouped irregularly so as to represent the photographic 5 lights and shades which it is desired to reproduce.

It is preferable that only those portions of emulsion be hardened which are adjacent the carrier for the emulsion, which may be accomplished in various ways, some of which are disclosed in my copending applications for Letters Patent Serial No. 313,239, filed July 25, 1919, for a thin mounted sensitized emulsion; Serial No. 313,240, filed July 25, 15 1919, for process of making a contact transfer printing surface by complementary light; Serial No. 327,891, filed October 2, 1919, for potassium iodide formula for photographic processes, process of using same, and article 20 obtained thereby; Serial No. 332,806, filed October 23, 1919, for process of making a contact transfer printing surface with a colored emulsion, and among which may be mentioned the exposure of the sensitized 25 emulsion through its transparent carrier and the limitation of the depth to which the rays of exposure light penetrate by having the actinic rays of the exposure light and the emulsion complementary in color.

30 If desired the hardened emulsion may be fixed to remove the silver salts unaffected by light, and bleached to remove the black metallic silver. This may be done in well known manner, and while not necessary, is of advantage as it enables the operator to watch the effect of the coloring matter on the printing surface to which it is applied for carrying out the printing process.

40 The order of melting, bleaching, and fixing is not important and may be carried out in any order desired, although it generally is more convenient to fix, melt, and bleach, in the order named.

45 The printing of positives from the printing surface may be done by direct contact. The printing surface is exposed to the action of the desired coloring matter as by placing it in or carrying it through a liquid color bath. The colored surface then is placed in 50 contact, preferably under some pressure, with the substance on which the positive is to be made, as by a roller or by a squeegee action. As stated above, the printing surface prepared by my process receives and gives up 55 the coloring matter almost instantly as dis-

tinguished from other processes which take an appreciable length of time.

Natural color effects may be produced in well known manner, such for example as by exposure through color screens with subsequent treatment and manipulation to obtain 60 the desired results.

Many modifications of my invention will be apparent to those skilled in the art without departing therefrom or from the scope 65 of the claims, my invention not being limited to the embodiments thereof chosen for purposes of illustration but consisting of a process for forming a printing surface on a negative capable of acquiring and giving 70 up a desired color with great rapidity.

Having described one embodiment of my invention, what I claim is:

1. The process of forming a photographic record of lights and shades capable of use 75 as a transfer printing plate, which comprises developing an exposed photographic emulsion with a non-emulsion-hardening solution, exposing it to an actinic light, and then hardening portions of emulsion adjacent the 80 light affected sensitive content of the emulsion with an agent adapted to harden said emulsion by reaction with the light affected sensitive content of the emulsion, and with a neutralizing agent for said hardening 85 agent, the relative proportions of said hardening and neutralizing agents being such as to control selectively the effective area of influence of the hardening agent but to an extent less than the complete neutralization of 90 said hardening agent.

2. The process specified in claim 1 in which the sensitive content is a silver salt.

3. The process specified in claim 1 in which the hardening agent is pyrogallic acid. 95

4. The process specified in claim 1 in which the neutralizing agent is sodium sulphite.

5. The process specified in claim 1 in which the hardening agent is pyrogallic 100 acid and the neutralizing agent is sodium sulphite.

6. The process specified in claim 1 to which is added the step of removing the unhardened portions of emulsion subsequent to 105 said treatment.

In testimony that I claim the foregoing, I have hereunto set my hand this 30<sup>th</sup> day of September, 1919.

ROBERT JOHN.